

## UNITED STATES PATENT OFFICE

2,051,383

METHOD FOR THE ELIMINATION OF  
HANGING-DISTURBANCES IN SHAFT  
FURNACES

Wilhelm Lennings, Oberhausen, and Ernst Karwat, Grosshesselohe, near Munich, Germany, assignors, by mesne assignments, to Union Carbide and Carbon Corporation, a corporation of New York

No Drawing. Application February 4, 1935, Serial No. 4,982. In Germany February 5, 1934

2 Claims. (Cl. 75—41)

This invention relates to the operation of blast furnaces and has for its object the elimination of troubles due to the tendency of the charge of such furnaces to stick or "hang" in the shaft.

In shaft furnaces, for example, in the production of iron or phosphorus in the blast furnace or in the burning of cement clinkers, the operation is frequently violently disturbed in that the charge passes irregularly downward through the shaft and finally hangs. In the production of iron, in order again to start up a furnace which has so hung it is customary to blow with a colder blast after the hanging-disturbance begins. In other instances, for example, in the production of cement, this method cannot be employed because cold blast is ordinarily utilized from the start. In such a cast it is usual to combat the disturbance by means of intensely cooling the shaft walls or by briquetting the fuel together with the fines of the charge.

We have discovered that such hanging disturbances in shaft furnaces can be eliminated in a surprisingly easy manner by increasing the oxygen concentration in the furnace blast. This discovery could in no way be foreseen because in many ways, particularly in regard to the distribution of heat between the hearth and shaft, an enrichment of the blast with oxygen has directly opposite results from those desired. Thus, the idea of utilizing oxygen-enriched blast for the same purposes for which hot blast is used is well known. It has, for example, been proposed to utilize oxygen-enriched blast in place of high blast temperatures in those instances in which a particularly powerful smelting effect is required in the hearth, or where the normal smelting temperature is too low, such for example as in the production of a high melting point strongly basic slag of the composition of Portland cement or when the furnace threatens to freeze up.

Inasmuch as it is known that an increase in the blast temperature does not reduce hanging disturbances but rather tends to increase them, it was in no way obvious that the enrichment of the blast with oxygen, which in regard to the smelting action has the same effects as hot blast, would eliminate hanging disturbances contrariwise to the effect of hot blast.

Oxygen enrichment of the blast in accordance with the practice of the present invention has the advantage in comparison with operation uti-

lizing ordinary cold blast that while the blast heat introduced into the hearth remains approximately the same, the temperature in the hearth and consequently the available quantity of heat are increased as compared to normal operation. As a result there is a lessening of the dangerous consequences of hanging, such for example as the sudden descent of the shaft contents into the hearth whereby there may result a too intense cooling of the iron and slag in the hearth and displacement of the slag so that it comes into contact with the ore charge. Such harmful disturbances are decreased to a much greater extent by increasing the oxygen concentration of the blast than by the utilization of a colder blast.

The explanation for the similarity of the effects of cold blast and oxygen enrichment in the elimination of hanging disturbances may be sought in the fact that both of these methods result in an increase in the volume of oxygen passing through the blastpipe-cross section per unit of time. Naturally, it is also possible, for the elimination of hanging difficulties, to reduce the temperature of the blast simultaneously with oxygen enrichment without departing from the spirit of my invention. Likewise, the utilization of oxygen enriched blast may be limited to such period as the furnace continues to hang and then continuing the operation with ordinary air as furnace blast. Sometimes, however, in a furnace which operates with difficulty, it will be advantageous to enrich the blast with oxygen continuously, in which case the concentration of oxygen may be increased to the desired extent and for such a period of time as may be necessary to overcome a tendency for the charge to hang.

We claim:

1. Method of overcoming the difficulties associated with the tendency of blast furnace charges to hang, which comprises increasing the oxygen content of the blast until the disturbance has been corrected.

2. In a blast furnace smelting process, the method of correcting a hanging of the charge, which comprises increasing the oxygen content of the blast, and decreasing the temperature of the blast, until the effects of the disturbance have been eliminated.

WILHELM LENNINGS. 50  
ERNST KARWAT.